

# United States Patent Office

2,777,765

Patented Jan. 15, 1957

1

2,777,765

## LOW MELTING CRUSHABLE TUNGSTEN ALLOY

John L. Benham, Lewiston, N. Y., assignor to Union Carbide and Carbon Corporation, a corporation of New York

No Drawing. Application October 11, 1955,  
Serial No. 539,925

7 Claims. (Cl. 75—122)

This invention relates to a refractory tungsten alloy, 15 and relates especially to a low melting, crushable ferrotungsten alloy composed of iron, tungsten and chromium.

It has long been known that tungsten alloys are generally distinguished by their unusual hardness and heat stability. Tungsten itself possesses the disadvantage that it requires an extremely high temperature, approximately 3370° C., for it to be fused and assimilated as an alloying ingredient in a molten metal bath. This objection has been overcome to some degree by combining the tungsten with a metal of lower melting point, such as iron, to form a ferrotungsten alloy, which is more easily fusible than tungsten alone, and which therefore may be more readily converted into a molten state. A ferroalloy containing 30% tungsten is admirably suited for such purposes, since it has a melting point in the vicinity of only 1550° C.

Theoretically ferrotungsten alloys having 30% tungsten represent an excellent starting material for producing certain engineering alloys. However, 30% ferrotungsten alloy is very tough, and is virtually incapable of being crushed by normal means. In granular form, this ferrotungsten is admirably suited to be melted and formed into ingots, in accordance with the method described in U. S. Patents 2,191,479, 2,191,480 and 2,191,481. Were it commercially and practically feasible to crush these tungsten alloys, the problem of using them in crushed or granulated condition for alloying or other metallurgical purposes would be simplified.

It is, therefore, a principal object of the present invention to provide a ferrotungsten alloy which is adapted to be used in the production of the aforesaid ingots.

Another object of the present invention is to provide an improved ferrotungsten alloy having approximately the same or lower melting point than a ferrotungsten alloy containing about 30% tungsten, yet having a greater degree of crushability.

Yet another object of the present invention is to provide a new alloy of tungsten, chromium and iron that may be used in crushed or granulated condition as an alloy additive or for other metallurgical purposes.

I have discovered that by the addition of chromium to a ferroalloy of tungsten, a very remarkable increase in crushability can be obtained. This is a remarkable phenomenon in view of the fact that the melting point of my new and improved ferrotungsten chromium alloy is substantially lower than the 30% binary ferrotungsten alloy.

The alloy of the invention contains 26% to 33% tungsten, 25% to 32% chromium, and the remainder iron and incidental impurities. With the alloy may be associated carbon in significant amounts up to 1.0% of the alloy. Best results may be obtained with an alloy having the following proportions:

|                              | Percent   |
|------------------------------|-----------|
| W                            | 30.00.    |
| Cr                           | 29.00.    |
| C                            | 1.00 max. |
| Fe and incidental impurities | Balance.  |

2

Crushable tungsten alloys with the foregoing composition ranges generally have a melting point approximately between 1270° C. and 1325° C.

An obvious advantage of the alloy of the present invention is that no special technique is required in manufacturing it. The alloy may be produced in a conventional induction furnace by adding ferrotungsten alloy to a bath of substantially pure iron containing additions of either high or low carbon ferrochromium, the high purity iron being used primarily to limit the impurity content in the bath. The heat may be taken up to a temperature of approximately 1675° C., which is slightly above the melting point of the alloy, and poured at that temperature.

In order to indicate still more fully the nature of the present invention, the following test results are set forth, it being understood that the data is presented as illustrative only, and is not intended to limit the scope of the invention. Two alloys were tested, alloy I being a ferrotungsten alloy having approximately 10% chromium, and alloy II a specific composition typical of ferrotungsten alloys of the invention. Their analyses were as follows:

|    | Alloy I,<br>percent | Alloy II,<br>percent |
|----|---------------------|----------------------|
| W  | 29.53               | 30.42                |
| Fe | 56.07               | 36.13                |
| Cr | 10.14               | 30.74                |
| Si | 0.47                | 0.60                 |
| C  | 0.85                | 0.89                 |
| S  | 0.021               | 0.029                |
| P  |                     | 0.025                |
| N  |                     | 0.065                |

Each of the above alloys was comminuted in a conventional crusher to particle sizes capable of passing through a screen having two inch mesh openings. Alloy I was crushed with extreme difficulty, the crusher apparatus jamming several times during the course of operations. Only about 8% of alloy I was sufficiently reduced in size to pass through a screen having two inch openings, the smallest particle size produced being of the order of 1½ inches. The remaining portion of alloy I ranged in particle dimensions up to about 4 inches.

In contrast, 20 pounds of the alloy II of the invention 45 were crushed with ease to a maximum particle size of two inches, and further reduced to a maximum particle size of 3/32 inch (8 mesh size) in conventional crusher equipment. This crushed alloy was then milled for one hour with comparative ease to produce the following 50 results:

|                 | Screen Size<br>Tyler Series | Alloy II<br>Before<br>Milling | Alloy II<br>After Mill-<br>ing 1 Hr. |
|-----------------|-----------------------------|-------------------------------|--------------------------------------|
| Retained on     | Mesh                        |                               |                                      |
| Do.             | 8                           | 0.5                           | Nil                                  |
| Do.             | 20                          | 54.0                          | 1.0                                  |
| Do.             | 48                          | 26.0                          | 6.5                                  |
| Do.             | 100                         | 8.0                           | 22.5                                 |
| Do.             | 200                         | 5.0                           | 20.5                                 |
| Passing Through | 200                         | 6.0                           |                                      |
| Do.             | 325                         | 12.0                          |                                      |
| Do.             | 325                         | 37.5                          |                                      |

From the above it will be seen that low melting ferrotungsten alloys containing chromium in the indicated proportions are entirely suitable as engineering alloys, where fusibility and crushability are important considerations, and are adapted to be pulverized in conventional crusher apparatus to particles passing through 20 mesh screens. It should be noted, however, that for the chromium content to be effective in the alloy of the invention, it should be sufficiently high to impart ease of fusibility as well as the desired crushability.

What is claimed is:

1. An alloy containing 26% to 33% tungsten, 25% to 32% chromium, and the remainder iron and incidental impurities.
2. A mass of finely divided particles composed of the alloy defined by claim 1.
3. A low melting, crushable, ferrotungsten alloy containing 26% to 33% tungsten, 25% to 32% chromium, and the remainder iron and incidental impurities.
4. An alloy containing 26% to 33% tungsten, 25% to 32% chromium, and the remainder iron and incidental impurities, said alloy being further characterized in that its melting point lies approximately between 1270° C. and 1325° C. and has a greater degree of crushability than binary ferrotungsten alloys containing approximately the same amount of tungsten.
5. An alloy containing 26% to 33% tungsten, 25% to 32% chromium, up to 1.0% carbon, and the remainder iron and incidental impurities.

6. A ferrotungsten alloy required to fuse at a temperature approximately between 1270° C. and 1325° C., and having a low resistance to reduction in particle size, said alloy containing 26% to 33% tungsten; 25% to 32% chromium, and the remainder iron and incidental impurities.

7. A ferrotungsten chromium alloy adapted to be pulverized to particles smaller than 20 mesh size, and having a melting point between 1270° C. and 1325° C., said alloy containing approximately 30% tungsten, approximately 29% chromium, up to 1.00% carbon, and the remainder iron and incidental impurities.

References Cited in the file of this patent

UNITED STATES PATENTS

|           |            |               |
|-----------|------------|---------------|
| 1,357,550 | Fahrenwald | Nov. 2, 1920  |
| 1,471,326 | Copland    | Oct. 23, 1923 |
| 1,593,924 | Wirth      | July 27, 1926 |